

# UNITED STATES PATENT OFFICE.

FRANK L. RANDEL, OF NEW YORK, N. Y.

## SULFATED OIL.

1,374,607.

Specification of Letters Patent. Patented Apr. 12, 1921.

No Drawing.

Application filed December 11, 1919. Serial No. 344,136.

To all whom it may concern:

Be it known that I, FRANK L. RANDEL, a citizen of the United States, residing at New York, in the county of New York and State 5 of New York, have invented certain new and useful Improvements in Sulfated Oils, of which the following is a specification.

This invention relates to sulfated oils; and it comprises a method of producing materials of the nature of what is known as turkey-red oil or alizarin oil by the action of strong sulfuric acid on fatty oils wherein the mixture of oil and sulfuric acid is kept at a low temperature by the action of 10 suction or vacuum, the lowering of temperature being advantageously aided by the addition of more or less volatile inert material, such as gasoline or benzol, to the reaction mixture; all as more fully hereinafter set 15 forth and as claimed.

On reacting upon various fatty oils with sulfuric acid at a low temperature compositions are produced containing the elements of the acid and of the oil, these compositions 20 being sometimes called sulfonated oils and sometimes sulfated oils. They are also known as "soluble" oils and greases. Ordinarily, castor oil is the oil employed and the product is then known as turkey-red oil 25 or alizarin oil. For this purpose castor oil has the advantage that its reaction with sulfuric acid is a fairly clean one; there is very little charring or oxidation at the expense of the acid if the temperature is kept at a 30 reasonably low point, say, below 35° C. The price of castor-oil is, however, relatively high and it is one of the objects of the present invention to produce similar materials 35 with the use of other and cheaper vegetable 40 and animal oils, not generally used for this purpose. Most of these oils in contact with sulfuric acid, char, oxidize or discolor at temperatures at which castor oil gives a clean action. The action of the acid upon 45 the oils is, relatively speaking, violent and is attended with development of heat. Since heat accelerates the action, if charring or browning starts in at any point, it is apt to spread rapidly throughout the mass. 50 Efforts have been made to obviate the effects of this development of heat to an extent allowing the use of cheap oils by special apparatus having water cooled stirrers, walls, etc.; but even with such apparatus, if it is 55 of any size, it is difficult to prevent localized initiation of heat and charring somewhere

in the mass. In sulfating these oils it is absolutely necessary that there be no opportunity for initiation of violent action.

The first or sulfating action of the acid on 60 the oil is attended with production of water ( $H_2O$ ) and this water reacts with excess of acid at the point of formation, developing a high temperature.

In the present invention I obviate the 65 effects of the development of heat and prevent any localization by the simple expedient of performing the mixing operation under a vacuum or strong suction. In so doing, water and other volatile bodies are 70 evaporated with development of a cooling effect on the entire mass. By the use of ordinary water cooling devices as auxiliaries to this evaporation cooling and vigorous stirring, the temperature of the mass may 75 be kept quite accurately at any point desired. The more vigorous the action of the acid on the oil the more energetic is the evaporation cooling; so that in the present invention, the action is, more or less, automatic and self-regulating; any tendency to 80 rise in temperature being at once repressed by increased evaporation and cooling. Evaporative cooling may often be advantageously increased, and particularly in the 85 case of the more delicate and sensitive oils and greases, by the expedient of adding inert volatile bodies such as hydrocarbons, like gasoline or benzol, or chlorinated materials such as carbon tetrachlorid, chloroform, chlorethylenes, ethylene chlorid, etc. Water itself may be added from time to 90 time during the action. As it is promptly re-evaporated it does not permanently dilute the material. Where these auxiliaries are 95 employed they may be mixed with the oil prior to sulfating or may be added from time to time in accordance with the observed progress of the reaction. It often happens that it is not desirable to preserve the same 100 temperature throughout the operation; it being, for example, often advantageous to start a little warm and finish at a lower temperature. In so doing the use of auxiliary volatile coolers gives a desirable independence of action; cooling not depending on the development of volatiles by the sulfating reaction. As such an auxiliary volatile body may be advantageously used the ordinary commercial "petroleum ether" or gasoline, 105 or I may use benzol. Whatever the auxiliary volatile material employed for cooling,

it may be condensed and regained in suitable condensing apparatus located beyond and connected to the pressure side of the suction apparatus. With the use of relatively small amounts of gasolene or benzol it is easy to keep the reaction mass at any low temperature even with oils or greases heating violently under the action of sulfuric acid. The greater the tendency for 5 the development of heat in the mass, the greater is the cooling. The whole mass, with efficient stirring apparatus, can be kept at substantially the same temperature with any oil; a temperature which can be readily 10 regulated by adjusting the amount of hydrocarbon to the degree of vacuum or suction employed.

In practising the present invention I may use any of the ordinary cheap commercial 20 fatty oils or oily fatty acids, such as cottonseed oil, cocoanut oil, palm oil, etc. The present process is applicable to the treatment of drying oils such as Chinese wood oil or tung oil, linseed oil, soy bean oil, etc., to 25 fish oils, commercial oleic acid, degras, corn oil, vegetable and animal greases, tallow, etc. Animal or vegetable oils which have been subjected to hydrogenation, or the so-called hardening, are easily handled by the 30 present process, these materials producing new substance of commercial possibilities. While many of these materials are very sensitive to the action of sulfuric acid, readily charring or browning with it, I find that 35 operating under the present invention they are readily applicable to the production of good, clean, light colored sulfated oils. Even castor oil though readily sulfated in the usual ways, gives better products when 40 treated under the present invention.

In one typical embodiment of the present invention I may mix four parts of ordinary cottonseed oil with six parts of strong sulfuric acid, the sulfuric acid being admitted 45 in a slow stream and the whole mass vigorously agitated. Prior to the operation the cottonseed oil may be let down with say, 10 per cent. of gasolene or benzol. On applying suction the mass can be cooled down 50 to any temperature which may be desired,

say 20 to 30° C. Cocoanut oil and palm oil may be treated in exactly the same way. As the reaction proceeds more or less of the volatile auxiliary cooling agent may be admitted from time to time so that temperatures are completely under control. Where an auxiliary cooling agent is used it must be a volatile body inert as regards the reaction but it is immaterial whether it is or is not miscible with the reaction mixture. 55

The products obtained under the present invention are chemically like the ordinary turkey red oils and soluble oils of commerce, though better in color; but their particular character of course depends more or less on 60 the particular oil used for sulfating. The process permits the use of practically any oily or fatty matter. The various products find application in the textile, paper, leather, paint, artificial leather, tanning, cutting oils, 65 soap, printing ink, dry cleaning and laundrying, etc., industries. They are good components of paints, typewriter inks, emulsions, etc.

The process permits a marked economy in 75 the amount of sulfuric acid necessary by reason of the automatic elimination of the water as fast as it is formed. In the ordinary processes of sulfating a large excess of acid is necessary to take up the water 80 formed in the reaction and preserve the needed strength of acid. Another important advantage of working under vacuum is the elimination of the oxidizing influence of air; this being particularly desirable in 85 working with drying or semi-drying oils.

What I claim is:—

1. The process of making a sulfated oil which comprises mixing a fatty or oily material of fatty nature with sulfuric acid 90 under vacuum producing conditions.

2. The process of making sulfated oily products which comprises mixing a fatty or oily material of fatty nature with sulfuric acid under vacuum conditions and in the 95 presence of an inert volatile cooling body.

In testimony whereof, I affix my signature.

FRANK L. RANDEL.